

Aug. 27, 1935.

W. GÖDECKE

2,012,465

THERMOCOUPLE OF HIGH ELECTROMOTIVE FORCE

Filed June 20, 1932



INVENTOR  
William Gödecke  
BY   
ATTORNEY

## UNITED STATES PATENT OFFICE

2,012,465

## THERMOCOUPLE OF HIGH ELECTRO-MOTIVE FORCE

Wilhelm Gödecke, Hanau-on-Main, Germany

Application June 20, 1932, Serial No. 618,112  
In Germany June 20, 1931

10 Claims. (Cl. 136—5)

This invention relates to thermocouples and aims at providing improved thermocouples of high electromotive force and thus rendering possible the use of very cheap measuring instruments which possess a low sensitiveness.

So far as thermocouples having limbs made of noble metals are concerned, the Le Chatelier couple has hitherto been most generally used, this alone having a measuring range up to 1600° C. The E. M. F. of this couple is, however, so small that it is necessary to use very highly sensitive measuring instruments which are very expensive.

The E. M. F. of thermocouples made from base metal components, such for example as constantan- and chrome-nickel couples and the like, is substantially greater, but their measuring ranges only extend up to about 900—1000° C., so that the extent to which they can be used is limited.

For a long time, therefore, attempts have been made to find thermocouples which, like the Le Chatelier couples, are suitable for temperatures up to about 1600° C. but which owing to increased E. M. F. can be connected to less sensitive and, therefore, more accurate and cheaper measuring instruments, and which enable measuring instruments of substantially higher total resistance to be used with particular accurate measurements.

It has been found that couples of higher E. M. F. and substantially higher heat resistance can be produced by making one limb from platinum or one of the platinum metals such as rhodium or of an alloy thereof, and the second limb from an alloy containing platinum and rhenium.

Even with rhenium contents of about 3%, such a couple has a substantially higher E. M. F. than one with limbs containing respectively platinum and platinum and rhodium. In general the rhenium may amount to between 3 and 15% of the total alloy, while it may advantageously be about 10%. Rhenium contents outside these limits may, however, sometimes be used.

Tests have shown that in comparison with the E. M. F. of 16.6 millivolts at 1600° C. produced by the Le Chatelier couple, the E. M. F. of a couple according to the invention and having a limb containing about 10% rhenium in addition to platinum is 45 millivolts, while an increase of the rhenium content leads to an increase in the E. M. F. to 60 millivolts.

By alloying further metals, such as rhodium, iridium, iron, nickel or cobalt, to the platinum-rhenium alloy, besides increasing the sensitivity and heat-resistance, this has the further advantage that the strong tendency of the platinum

metals to recrystallization can be avoided. Thus, for example, an addition of 3% rhodium is enough to prevent the alloy becoming brittle owing to recrystallization. A limit is set to the amount of further elements which may be added by the resultant increase in the specific resistance.

The heat resistance of the couples can be increased further if rhodium is included in the second limb. Thus for example thermocouples in which one limb contains rhodium and platinum and the other platinum and rhenium are more heat-resistant than those in which one limb consists of platinum alone and the other of platinum and rhenium.

With the use of a rhodium limb besides a platinum-rhenium limb, the heat-resistance is increased still further, that is to say up to about 1800° C., but in this case the E. M. F. is somewhat smaller and amounts to about 25 millivolts at 1600° C.

It has further been found that the combination of one limb made of a platinum-rhenium alloy with another limb made of palladium gives a thermocouple which has an E. M. F. at temperatures of 1000° C., and over which lies uniformly about 15 to 20 millivolts higher than that of a combination consisting of platinum on the one hand and platinum-rhenium on the other hand. The use of palladium for the second limb also makes the thermocouple cheaper, because the much smaller specific weight of palladium makes possible a reduction in the weight of the limb in comparison with a platinum limb.

It has also been found that, in thermocouples of the kind described so far in this specification, the rhenium of the platinum-rhenium alloy to be used for one limb can be replaced by metals which are adjacent to rhenium in the periodic system and especially by those of the fifth and sixth groups of the periodic system. Thermocouples of which one limb consists of platinum or palladium or another platinum metal while the second limb consists of platinum and a metal of the said kind instead of rhenium have proved to be remarkably efficient. The following metals in particular can be used instead of rhenium, viz.—vanadium, niobium, tantalum, molybdenum, tungsten, uranium and manganese. The amount of each of these metals which can be used largely depends upon the metal and upon the extent of which it can be worked, and these amounts vary between about 0.5 and 15%, and preferably between 3 and 10%. Amounts which have been found suitable are, for example, between about 50

1 and 4% vanadium, between about 2 and 10% molybdenum, and from 3 up to about 7% manganese.

5 The E. M. F. of such thermocouples, when one limb is made of platinum and the other of an alloy as described are as follows at 1200° C.—

|    | Composition of the alloy | E. M. F. |
|----|--------------------------|----------|
| 10 | Platinum +7% tantalum    | 23 m.v.  |
|    | Platinum +2.5% vanadium  | 30 m.v.  |
|    | Platinum +7% molybdenum  | 24 m.v.  |
|    | Platinum +9% tungsten    | 36 m.v.  |

15 The risk of oxidation due to the base metal character of the metals such inter alia as tungsten and molybdenum, as well as the volatility of the resultant oxides and any absorption or taking up of gas by the wires of the thermocouples, can be avoided if that limb which consists of an alloy of platinum with the said easily oxidizable metals is enclosed in a non-metallic, preferably gas-tight, material. Examples of suitable materials are highly fire-resistant porcelain, quartz and the like. 20 In order to prevent the access of oxygen to the enclosed wire, the latter may advantageously be fused into the material. Preferably a ceramic tube is used to encase the wire and the space within the tube around the wire is evacuated or 25 charged with an inert harmless gas such as nitrogen. The inert gas filling may be under normal or reduced pressure.

30 Thermocouples in which at least the limb containing an oxidizable metal of the said kind is protected as described above have proved uniform and constant in continuous operation with high E. M. F., even at high temperatures such as 1200 to 1400° C.

35 If a limb of one of the said alloys of platinum with a base metal is combined with a palladium limb instead of a platinum limb, the thermocouples have substantially higher E. M. F. In general the increase in E. M. F. at 1200° C., relatively to that of a thermocouple having the second limb of platinum, is about 15 millivolts.

40 When a palladium limb is used it has been found to be particularly advantageous to encase it gas-tightly in a ceramic material in the way described above, in order to counteract the tendency of palladium to take up gas on being maintained for some time at a high temperature and thus to bring about variations in the E. M. F. curve 45 of the couple.

45 If both limbs are encased gas-tightly, combinations such as palladium-platinum-tungsten or palladium-platinum-molybdenum have proved to be completely resistant. Such thermocouples, owing to their high E. M. F., have the substantial advantage that cheaper and less sensitive measuring instruments can be used for indicating the 50 E. M. F. than has been possible hitherto with noble metal thermocouples.

55 The drawing shows in cross section a thermocouple according to my invention.

In the drawing, 2—2 represent the two limbs of the thermocouple, which are encased in a covering element 4 of refractory material such as porcelain or quartz. The covering may be closed at its lower end by a sealing element 6 of insulating material of any suitable type.

60 The use of heat-resistant alloys with rhenium, which also have the property of not being attacked, affords in addition to the large range over which they can be employed, the substantial advantage that cheap, i. e. measuring instruments of low sensitiveness can be used, and this has not hitherto been possible with noble metal thermocouples.

65 What I claim is:

1. A thermocouple one limb of which consists essentially of a metal of the platinum group while the other consists essentially of platinum and rhenium.

2. A thermocouple one limb of which consists essentially of platinum and the other essentially of an alloy of platinum with rhenium.

3. A thermocouple one limb of which consists essentially of palladium while the other consists essentially of platinum and rhenium.

4. A thermocouple one limb of which consists essentially of a metal of the platinum group and the other essentially of an alloy of platinum with rhenium containing from 3 to 15% of rhenium.

5. A thermocouple one limb of which consists essentially of a metal of the platinum group and the other essentially of an alloy of platinum containing about 10% of rhenium.

6. A thermocouple one limb of which consists essentially of a metal of the platinum group while the other consists essentially of platinum and rhenium, to which a metal selected from the group consisting of rhodium, iridium, iron, nickel and cobalt is alloyed which is capable of preventing recrystallization.

7. A thermocouple one limb of which consists essentially of a metal of the platinum group while the other consists essentially of platinum and rhenium, to which a metal selected from the group consisting of iridium, iron and nickel is alloyed which is capable of preventing recrystallization.

8. A thermocouple one limb of which consists essentially of a metal of the platinum group while the other comprises essentially platinum, rhenium and rhodium.

9. A thermocouple one limb of which consists essentially of a metal of the platinum group while the other consists essentially of platinum, rhenium and substantially 3% of rhodium.

10. A thermocouple comprising two limbs the major portion of one of which limbs consists of a platinum metal and the major portion of the other of which limbs consists of platinum and rhenium.

WILHELM GÖDECKE.